

## UNITED STATES PATENT OFFICE

MAX HAGEDORN, OF DESSAU IN ANHALT, OTTO REICHERT, OF DESSAU-ZIEBIGK IN ANHALT, AND EUGEN GUHRING, OF DESSAU IN ANHALT, GERMANY, ASSIGNEES TO I. G. FARBENINDUSTRIE AKTIENGESELLSCHAFT, OF FRANKFORT-ON-THE-MAIN, GERMANY

## ELECTRIC INSULATING MATERIAL

No Drawing. Application filed January 31, 1930, Serial No. 425,056, and in Germany February 13, 1929.

Our present invention relates to new insulating materials for electric purposes, and more particularly to such materials as are composed of a cellulose derivative.

5 We have found that mixed cellulose esters of lower fatty acids are particularly suited for use in the manufacture of electric insulating materials without the addition of considerable quantities of heterogeneous substances. We may use for the said purpose a mixed ester of cellulose which contains simultaneously in any combination radicals of different lower fatty acids, that is to say, of the acids containing up to 5 carbon atoms:—acetic acid, propionic acid, butyric acid, valeric acid. We prefer to use such a mixed ester which contains the radicals of two lower fatty acids, however, those esters derived from more than two acids are meant 10 to be included within our invention. The said cellulose esters may be employed as primary esters or they may be subjected to a hydrolyzing process.

15 Of the great number of mixed esters of lower fatty acids, we prefer to use a cellulose derivative which contains the acetic acid radical in addition to another lower fatty acid radical. Such a mixed ester has both 20 the good mechanical properties of the cellulose acetate and a high stability towards saponifying agents. Cellulose acetate butyrate has proved to be especially suitable. Thus, for instance, a foil of 0.13 mm. thickness of a cellulose acetate-butyrate containing in the molecule 1½ molecular proportions of the acetate acid radical and 1½ molecular proportions of the butyric acid radical 25 calculated on  $C_6H_{12}O_6$  has a sparking potential or dielectric strength of about 16000 volts and of 9500 volts after having been immersed in distilled water for 200 hours.

The superiority of our new insulating materials over those prepared from cellulose

|                                                                                    | Commercial cellulose-acetate | Cellulose acetatebutyrate | 50 |
|------------------------------------------------------------------------------------|------------------------------|---------------------------|----|
| Thickness.....                                                                     | 100 $\mu$                    | 90 $\mu$                  |    |
| Sparkling potential of the air-dry product.....                                    | 6, 8 kilovolts               | 11, 4 kilovolts           |    |
| Sparkling potential after having been immersed for 48 hours in water at 20° C..... | 2, 2 kilovolts               | 8, 2 kilovolts            |    |
| Sparkling potential of the product in transformer oil.....                         | 7, 65 kilovolts              | 10, 9 kilovolts           | 55 |
| Sparkling potential after having been immersed for 24 hours in oil at 100° C.....  | 9, 6 kilovolts               | 12, 1 kilovolts           |    |
| Dielectric constant.....                                                           | 5, 62                        | 2, 99                     |    |

60 The mixed cellulose esters can be worked up in such a manner that paper or fabrics are impregnated with their solutions and are used for taping cables. The materials thus prepared, may, however, also be used for other insulating purposes. There can likewise be used for insulating purposes layers of the mixed cellulose esters alone by covering the cables, surfaces or the like to be insulated with a lacquer of these cellulose derivatives.

65 We may incorporate into the new insulating substance any of the additions which are known in the industry dealing with the manufacture of electric insulating materials such as, for instance, filling materials, pigments, dyes, natural or artificial resins, plastifying or softening agents or another cellulose derivative.

70 For the manufacture of our new insulating materials, we may use the solvents known in the art; it is advisable, however, to avoid the use of chlorinated hydrocarbons, which split off hydrochloric acid in the course of time. When forming the insulating body with the application of heat and pressure the use of a solvent may be dispensed with.

75 The following examples serve to illustrate our invention:—

80 Example 1.—A solution of cellulose ace-

tate-butyrate (1½ mol. of acetic acid and 1½ mol. of butyric acid) in acetone is cast in the known manner so as to form a film of a strength of 80 to 100  $\mu$  and the film cut into 5 tape of a breadth of 25 mm. The electric cables are wound with this tape in a taping machine.

Example 2.—A solution of cellulose-mono-acetate-dipropionate in a mixture of alcohol, 10 benzene and acetone in a proportion of 1:1:7 is cast to foils of a strength of 10 to 20  $\mu$ . The foils are used in the known manner together with metallic foils for preparing high tension condensers.

15 Numerous other embodiments are possible and we contemplate as included within our invention all such modifications and equivalents as fall within the scope of the appended claims.

20 What we claim is:—

1. An electric insulator comprising a compound selected from the group consisting of a cellulose acetate-butyrate and a cellulose acetate propionate.

25 2. An electric insulator comprising cellulose acetate butyrate.

3. An electric insulator comprising cellulose mono acetate dipropionate.

30 In testimony whereof, we affix our signatures.

MAX HAGEDORN.  
OTTO REICHERT.  
EUGEN GUHRING.

35

40

45

50

55

60

65